

# UNITED STATES PATENT OFFICE.

FREDERICK WALTON, OF HEATHAM HOUSE, TWICKENHAM, COUNTY OF MIDDLESEX, ENGLAND.

## MANUFACTURE OF PANELS, SLABS, AND OTHER ARTICLES FROM OXIDIZED OIL.

SPECIFICATION forming part of Letters Patent No. 249,428, dated November 8, 1881.

Application filed July 26, 1881. (Specimens.) Patented in England July 19, 1880.

To all whom it may concern:

Be it known that I, FREDERICK WALTON, a subject of the Queen of Great Britain, residing at Heatham House, Twickenham, in the county of Middlesex, England, have invented a certain Improvement in the Manufacture of Panels, Slabs, and other Articles from Oxidized Oil, (for which I have received Letters Patent in England, No. 2,975, dated the 19th day of July, 1880;) and I do hereby declare that the following is a full, clear, and exact description of the invention, which will enable others skilled in the art to which it appertains to make and use the same.

15 This invention has for its object novel or improved applications of oxidized-oil or solidified-oil compositions to panels, moldings, and articles requiring an impermeable molded surface.

According to my invention I apply or make 20 use of oxidized or solidified oil compositions to give an ornamental or smooth, impermeable, and durable molded surface to panels or moldings for furniture, and panels or slabs to form ornamental parts of writing-desks, boxes, and 25 such like articles; and I produce ornamental slabs or sheets for the decoration of shops, and for the exhibition of maps or advertisements in a decorative form, and ornamental letters and signs for shop-windows and the like. For 30 the purpose of applying the oxidized or solidified oil composition I employ engraved metal dies or rollers.

35 A suitable composition may be prepared as follows: A cement is first made consisting of oxidized oil, four hundred-weight; kauri gum, twenty-one pounds; resin, one hundred-weight. These materials are mixed in steam-heated pans.

40 The composition for molding consists of cement, (as above,) forty-eight pounds; wood fiber, forty-eight pounds; white lead, six pounds; Venetian red, three pounds. These materials are combined in radial mixing-machines. The color can be altered to suit the 45 purpose required.

The composition is applied to the panel or article when in a plastic state, and considerable pressure is employed. Afterward the ar-

ticles are hardened off by exposure to a moderate heat for a considerable time. The panels, 50 slabs, moldings, ornamental letters, or like articles for receiving the impermeable molded surface will usually be of wood; but in some cases other hard and solid materials may be conveniently employed. In this way, also, I 55 coat or surface articles requiring protection from moisture or the weather. Thus wheels are sometimes made with the central portion of compressed paper; and the most serious objection to which such wheels are liable is that 60 the block is not impermeable. This objection I wholly remove by the application, as above described, by means of dies and pressure, of a skin or surface of oxidized or solidified oil composition. The said composition in a plastic 65 state is molded onto the block and in such a manner as to completely incase it, so as to exclude the access of moisture to the paper material. Other perishable articles liable to be injured by moisture may be similarly protected. 70 Thus cords of fibrous material may be inclosed in an impermeable sheath. Where desired, ornaments may be produced upon the surface by means of dies or rollers at the same time that the impermeable skin or surface is molded up 75 on it or subsequently.

Having thus described the nature of my said invention and the manner of performing the same, I would have it understood that I claim—

1. The new manufacture herein described, 80 consisting of panels, slabs, moldings, ornamental letters, signs, and other articles of wood or other hard and solid material having compositions of oxidized or solidified oils, hereinbefore set forth, to give an impermeable molded 85 surface, substantially as described.

2. The hereinbefore-described advertising-sheet or similar article of wood or other hard and solid material, having an impermeable molded surface formed of the oxidized or solidified oil composition, substantially as described. 90

FRED. WALTON.

Witnesses:

JOHN DEAN,

J. WATT,

Both of 17 Gracechurch Street, London, E. C.